

# UNITED STATES PATENT OFFICE.

OSCAR MÜLLER, OF COLOGNE, GERMANY, ASSIGNOR TO THE FIRM OF RHEINISCHE KUNSTSEIDE-FABRIK, AKTIENGESELLSCHAFT, OF COLOGNE-ON-THE-RHINE, GERMANY.

## CELLULOSE SUBSTITUTE.

No. 930,874.

Specification of Letters Patent.

Patented Aug. 10, 1909.

Application filed February 1, 1906. Serial No. 299,048.

*To all whom it may concern:*

Be it known that I, OSCAR MÜLLER, a subject of the King of Prussia, residing at Cologne-on-the-Rhine, Krefelderstrasse 24, Germany, have invented certain new and useful Improvements in Cellulose Substitutes.

My invention relates to the production of a cellulose substitute and particularly to a process of obtaining the same from cotton seed shells and other cotton waste.

The waste products to which my invention relates comprise cotton seed shells with or without adhering fibers and linters as they come from the shelling processes, and also to the fibers in the dust of the cotton mill. These waste products have heretofore either been thrown away or used as fuel, though of little calorific value.

My investigations have revealed that these shells contain not only a valuable cellulose substitute commercially obtainable by a suitable chemical process but also a valuable dye. The seed hairs and linters of the above mentioned waste have been discovered to be valuable not only for spinning purposes but for practically all the other purposes as well, for which the staple fibers of cotton are generally employed and indeed in specific instances are to be preferred thereto. I have found that this cellulose structure is not only suitable for nitrating purposes, but is extremely well adapted for the manufacture of paper, artistic threads, substitute for caoutchouc or the like, and in the production of cellulose derivations of all kinds. Its value for these purposes is enhanced by the remarkably pure condition in which it is obtained. A suitable process by which this may be accomplished is given herewith.

For example, if necessary, the shells are first passed through a suitable machine to effect as far as possible a mechanical separation of the linters and seed hairs from the shell. This is not essential however inasmuch as the chemical treatment which follows will of itself effect this separation, although the preliminary mechanical treatment is preferred. The shells are then heated, preferably boiled for some hours with steam, in open vats, and under pressure if necessary, in an alkaline lye, (for example, sodium hydrate of a strength of from 3% to 10° Bé according to the origin of the cotton seed, as the case may be). After this treatment is completed the boiling

fluid is drawn off and the remaining mass washed with water. A permanganate bath at about 20° C. follows, lasting for about 30 minutes. This bath is preferably agitated, for instance by blowing through a stream of air, oxygen or the like. If potassium permanganate be used for the bath, a suitable strength is obtained by adding 1 kilo of potassium permanganate to 1000 liters of aqueous solution. Without an intervening washing the mass is then subjected to a sulfurous acid bath containing in 1000 liters about 6 kilos of hydrochloric acid (of about 20° Bé) and about 14 liters bisulfite solution for instance bisulfite of soda (of about 35° Bé). The action of this bath may be assisted by heating it to about 40° C. and continued until a plastic translucent mass results. This transparent mass may be perfectly bleached by a subsequent chlorin bath containing 3 to 4 per cent. effective chlorin. The temperature and duration of this bath are regulated to prevent any decomposition of the shell substance. If by chance this should happen however, the substance may be extracted again by precipitation.

If the mass treated according to the above process contains large quantities of staple cotton fiber or linters then the undesirable chlorin bath may generally be omitted. In such cases furthermore, a weaker alkali bath may be used, for example, of a strength of only 1° or 2° Bé. The sulfurous acid bath of less strength, say half strength, may be used successfully.

During the alkali treatment a quantity of soluble matter in the shells is dissolved in the alkali lye, including the coloring matter or dye above mentioned, in quite conspicuous quantities, and also the resinous or wax-like binding substances of the shell. When this lye is neutralized these matters are obtained as a deposit. A colored lac may be secured from this, which can be used in suitable solvents (such as ether, turpentine, alcohol, benzine, etc.) as lacquer or the like. These solutions are very valuable as a paint for glass or metal since the substance adheres very fast to glass and does not corrode metals.

After the above mentioned resins and dye stuff have been removed from the mass under treatment there remain not only linters which may have adhered to the shell, and

the seed hairs but also the pith cells and woody fibers of the shell which form the cellulose structure proper.

While during the subsequent steps set out in the process all of these substances are customarily permitted to remain together in the baths it is possible to separate the cellulose structure from the fibers (*i. e.* the linters and seed hairs) during the latter part of the treatment, and obtain a practically pure cellulose if desired. This separation is readily accomplished by sieves or by decanting since the cellulose substance tends to settle as a deposit while the fibrous structure is suspended in the bath. It should be noted however for many purposes such as the production of artificial silk and for nitrating purposes, such a separation may not be deemed necessary.

In connection with the above process it is to be understood that the hot alkali lye treatment does not and is not intended to affect the mercerization or hydratization of the cellulose substance. Furthermore the process may be modified by subjecting the mass to treatment in alternating chlorin baths after the boiling in the alkali lye. One of these baths should contain about 3 to 4 per cent. effective chlorin while the other should be much weaker say from one-fifth to one-tenth this strength. Both baths are maintained at room temperature or slightly higher (say 40° C.). The baths may be made by dissolving chlorid of lime in water and adding thereto a corresponding solution of an alkaline carbonate (of sodium carbonate or bicarbonate) preferably supersaturated. In practice it is preferable to boil the carbonate solution and after cooling to add it to the cold chlorid of lime solution. A

clear serviceable chlorin bath is thus obtained. If these chlorin baths contain an alkali (*e. g.* soda) the cellulose is obtained from the shells with safety and ease, and further by this treatment the linters and seed fibers are transformed into a pure white soft fiber product which may be used for practically all the purposes for which the staple cotton fiber is employed.

The treatment with the chlorin baths is preferable to that first mentioned since the different kinds of bath are fewer in number, while the dye matter is extracted from the shells in usable form and the essential shell substance is obtained in cellulose form adapted for chemical treatment for commercial purposes as in the first mentioned method.

Other processes may be devised for accomplishing the same end and I do not limit myself to the processes set forth.

I claim as my invention:

1. A cellulose substance comprising cotton seed shells from which the binding materials and cotton fibers have been eliminated.

2. A cellulose substance comprising cotton seed shells from which the binding materials, dye substances and cotton fibers have been eliminated.

3. A cellulose substance comprising the shell substance of cotton seed from which the binding materials have been eliminated, substantially as described.

In testimony whereof I have signed my name to this specification, in the presence of two subscribing witnesses.

OSCAR MÜLLER.

Witnesses:

BESSIE F. DUNLOP,  
LOUIS VANDORN.